



US006066375A

# United States Patent [19]

Shanton

[11] Patent Number: 6,066,375

[45] Date of Patent: May 23, 2000

[54] COATED PAPERBOARD AND PAPERBOARD CONTAINERS HAVING A MICROWAVE INTERACTIVE LAYER WHICH EMITS NONE OR VERY LOW AMOUNTS OF BENZENE IN MICROWAVE APPLICATIONS

[75] Inventor: Kenneth J. Shanton, Neenah, Wis.

[73] Assignee: Fort James Corporation, Deerfield, Ill.

[21] Appl. No.: 08/835,700

[22] Filed: Apr. 10, 1997

[51] Int. Cl.<sup>7</sup> C08K 3/08

[52] U.S. Cl. 428/35.7; 428/34.2; 428/35.3

[58] Field of Search 428/34.2, 35.3

## [56] References Cited

### U.S. PATENT DOCUMENTS

|           |         |                     |         |
|-----------|---------|---------------------|---------|
| 4,518,768 | 5/1985  | Scheurer et al.     | 528/483 |
| 4,721,500 | 1/1988  | Van Handel et al.   | 493/152 |
| 4,900,809 | 2/1990  | Tazi et al.         | 528/497 |
| 4,962,185 | 10/1990 | Tazi et al.         | 528/497 |
| 4,992,517 | 2/1991  | Tazi et al.         | 526/209 |
| 5,049,714 | 9/1991  | Beresniewicz et al. | .       |
| 5,079,083 | 1/1992  | Watkins et al.      | .       |
| 5,118,747 | 6/1992  | Pollart et al.      | .       |
| 5,231,269 | 7/1993  | Oku et al.          | .       |
| 5,278,377 | 1/1994  | Tsai.               | .       |
| 5,308,945 | 5/1994  | VanHandel et al.    | .       |

5,338,911 8/1994 Brandbert et al. .  
5,349,168 9/1994 Wilen. .

Primary Examiner—Charles Nold

## [57] ABSTRACT

An improved, coated microwaveable paperboard or container useful for forming substantially rigid food containers such as plates, bowls, trays and the like and a process from producing the improved, coated paperboard is provided. The microwaveable paperboard and food containers, at a temperature in excess of 430° F. evolves less than 0.1 milligrams of benzene per square inch, preferably less than 0.04 milligrams. Said paperboard and food containers are produced from a sized paperboard blank wherein a base coat and top coat comprise a mixture of an inorganic pigment and aliphatic copolymers. A base coat comprising an aliphatic latex and a pigment is applied directly to the paperboard, and a top coat comprising the same or different aliphatic polymer latex and a pigment is applied directly to the base coat to form the coated containers. Microwave susceptor layers are coated on the top coat. These containers are used to microwave and brown food at temperatures in excess of 430° F. without evolving more than 0.1 milligrams of benzene per square inch of the container surface. The coated containers are also characterized by improved grease, oil, and cut resistance, improved varnish gloss, enhanced smoothness, and improved printing quality.

47 Claims, 16 Drawing Sheets



Bowl with discontinuous  
Microwave Susceptor Layer



FIG. 1B



FIG. 1C



FIG. 1A

Bowl with continuous  
Microwave Susceptor Layer



FIG. 2B

SEE FIG. 2A



FIG. 2C



FIG. 2A

## Canister



FIG. 3A



FIG. 3B

## Compartmented Plate



**FIG. 4A**



**FIG. 4B**

## French Fries Sleeve



FIG. 5

Rectangular Take-Out Container



FIG. 6A



FIG. 6B

## Hamburger Clamshell



FIG. 7A



FIG. 7B

## Cup



FIG. 8A



FIG. 8B

## Cup



FIG. 9A



FIG. 9B

## Food Bucket



FIG. 10A



FIG. 10B

Food Container  
with Microwave Susceptor Layer



FIG. I A



FIG. I B

Manufacture of basestock



FIG. 12

## Manufacture of press formed articles



FIG. 13



FIG. 14



FIG. 15

Lamination of Microwave Susceptor film to the  
coated web and press-forming of the article



FIG. 16

**COATED PAPERBOARD AND PAPERBOARD CONTAINERS HAVING A MICROWAVE INTERACTIVE LAYER WHICH EMITS NONE OR VERY LOW AMOUNTS OF BENZENE IN MICROWAVE APPLICATIONS**

**BACKGROUND OF THE INVENTION**

**1. Field of the Invention**

This invention relates to coated paperboards which, when converted to containers, can be used in microwave applications without emitting unacceptable amounts of benzene. Particularly, this invention relates to containers including a microwave interactive layer wherein at a microwave cooking temperature of about 430° F. or more, less than 0.1 milligrams of benzene are evolved per square inch of the container surface.

**2. Background**

Disposable paper containers, such as plates, trays, bowls, airline meal containers and cafeteria containers, are commonly produced by pressing flat paperboard blanks into the desired shape between appropriately shaped and heated forming dies. Various protective coatings are typically applied to the blanks before forming to make the resulting paperboard containers moisture-resistant, grease-resistant, more readily printable, etc. Often, printing is also applied to the top surface for decoration. Large numbers of paper products are produced by this method each year. These products come in many different shapes and sizes, including round, rectangular, and polygonal.

When a container is made by pressing a flat paperboard blank, the blank must contain enough moisture to make the cellulosic fibers in the blank sufficiently plastic to permit it to be formed into the desired three-dimensional container shape. During the pressing operation, most of this moisture escapes from the uncoated bottom surface of the blank as water vapor. Suitable methods of producing paperboard containers from moistened paperboard blanks are generally described in U.S. Pat. Nos. 4,721,499 and 4,721,500, among others.

Many people prefer disposable containers which, when handled, produce a sense of bulkiness and grippability at least suggestive of the more substantial non-disposable containers which they replace. While a sense of bulkiness may be provided to some extent in styrofoam and thick pulp-molded containers, such containers suffer a number of drawbacks and cannot include a microwave interactive layer. For example, unlike pressed paperboard containers, styrofoam containers are often brittle and they are environmentally unfriendly because they are not biodegradable and melt under microwaved conditions. Also, styrofoam containers are not cut-resistant and it is difficult to apply printing to the surface of styrofoam containers. Additionally, because of their bulkiness, styrofoam containers take up large amounts of shelf space and are costly to ship. Pulp-molded containers similarly are not cut-resistant and have poor printability characteristics. Additionally, pulp-molded containers typically have weak bottoms. Pressed paperboard containers, however, are cut-resistant, readily printable, strong in all areas, and are far less bulky than styrofoam or pulp-molded containers and can include a microwave interactive layer.

The prior art paperboard containers have difficulty in meeting the new low benzene evolution standards set by the food processors and therefore cannot safely be used in microwave applications or include a microwave interactive layer since their coatings emit an unacceptable amount of

benzene. Benzene is a well known carcinogen and its contact with food should be minimal.

**SUMMARY OF THE INVENTION**

The object of the present invention is to provide paperboards and paperboard containers which emit a minimal amount of benzene under microwave food preparation conditions. This is particularly critical when the container includes a microwave interactive layer. Usually benzene emission is increased when microwave susceptor layers are coated on the paperboard and/or the paperboard container. Metalized polyesters are suitably formed as a microwave susceptor layer on the paperboard surface as shown in FIG. 1. Aluminum and nickel are suitable metals. The microwavable, food contact compatible, disposable, rigid and strong paperboards and paperboard containers of this invention at temperatures in excess of 430° F. evolve less than 0.1 milligrams of benzene per square inch, preferably less than 0.04 milligrams per square inch. This feature also holds true for the paperboard containers of this invention which include a microwave susceptor layer. These paperboard food containers comprise:

- (a) a sized paperboard blank having a basis weight suitable for a selected type of food container;
- (b) a base coat coating applied to one or both surfaces of the paperboard blank, the base coat coating comprising a mixture of an inorganic pigment and a polymer latex comprising aliphatic copolymers having the following monomers:



wherein R and R<sup>1</sup> may be the same or different aliphatic hydrocarbons having one to six carbon atoms and the ratio of (i) to (ii) is in the range of 1:100 to 100:1;

- (c) a top coat coating layer applied to the base coat coating layer, the top coat coating layer comprising an inorganic pigment and an aliphatic polymer latex comprising aliphatic copolymers having the following monomers:



wherein R and R<sup>1</sup> may be the same or different aliphatic hydrocarbons having 1 to 6 carbon atoms and the ratio of (i) to (ii) is in the range of 1:100 to 100:1.

In a preferred mode, both R and R<sup>1</sup> are methyl groups. The paperboard blank has suitably a weight in the range of about 100 to 400 lbs. per 3000 square foot ream and a caliper in the range of about 0.008 to 0.055 inches. In a suitable variant of this invention, sufficient moisture is introduced into the blank to produce a moisture content of about 4 to

12% by weight. These microwaveable containers are suitably prepared by sizing a selected paperboard suitable for use as a food container and applying a base coating to one or both surfaces of the paperboard blank. The base coat coating comprising a mixture of an inorganic pigment and a polymer latex comprising aliphatic copolymers having the following monomers:



wherein R and R<sup>1</sup> may be the same or different aliphatic hydrocarbons having one to six carbon atoms and the ratio of (i) to (ii) is in the range of 1:100 to 100:1, preferably the range of (i) to (ii) is 1:3 to 3:1;

A top coat coating layer applied to the base coat coating layer, the top coat coating layer comprising an inorganic pigment and an aliphatic polymer latex comprising aliphatic copolymers having the following monomers:



wherein R and R<sup>1</sup> may be the same or different aliphatic hydrocarbons having 1 to 6 carbon atoms and the ratio of (i) to (ii) is in the range of 1:100 to 100:1, preferably the range of (i) to (ii) is 1:3 to 3:1.

In a preferred embodiment, these paperboard containers include a microwave susceptible layer. This microwave susceptor layer is preferred for microwave cooking applications to give a brown appearance to cooked meat. Without the susceptor layer the food would also be cooked, but it would not have the pleasing brown color for meats preferred by consumers. At these high temperatures, in excess of 430° F., it is essential that evolution of benzene be kept below 0.1 milligrams per square inch of the container surface, preferably below 0.04 milligrams per square inch. According to our invention, we can tailor make the paperboard to control the evolution of benzene so that the total benzene evolution is below 0.03, 0.02, or 0.01 milligrams per square inch of the container surface.

The features of the invention which are believed to be novel are set forth with particularity in the appended claims. The invention, together with further objects, features and advantages thereof, may be best understood by reference to the following detailed description taken in conjunction with the accompanying drawings.

#### BRIEF DESCRIPTION OF THE DRAWINGS

FIGS. 1A, 1B and 1C are drawings of a bowl of this invention with a discontinuous microwave susceptor layer.

FIGS. 2A, 2B and 2C are drawings of a bowl of this invention with a continuous microwave susceptor layer.

FIGS. 3A and 3B are drawings of a canister of this invention with a microwave susceptor layer.

FIGS. 4A and 4B are drawings of a compartmented plate with a microwave susceptor layer.

FIG. 5 is a drawing of a French fry sleeve of this invention with a microwave susceptor layer.

FIGS. 6A and 6B are drawings of a rectangular take-out container of this invention with a microwave susceptor layer.

FIGS. 7A and 7B are drawings of a hamburger clamshell of this invention with a microwave susceptor layer.

FIGS. 8A and 8B are drawings of a cup of this invention with a microwave susceptor layer.

FIGS. 9A and 9B are drawings of a cup with handles of this invention with a microwave susceptor layer.

FIGS. 10A and 10B are drawings of a food bucket of this invention with a microwave susceptor layer.

FIGS. 11A and 11B are drawings of a food container of this invention with a microwave susceptor layer.

FIG. 12 is a drawing of a manufacturing operation of the paperboard basestock

FIG. 13 is a drawing of a manufacturing process for the manufacture of the containers of this invention starting with the coated paperboard web.

FIG. 14 is a flow diagram depicting the process for the manufacture of the paperboard of this invention.

FIGS. 15 and 16 are the flow diagrams depicting the conversion of the paperboard to the containers of this invention including the microwave susceptor layer.

#### DETAILED DESCRIPTION

The paperboards and containers of this invention evolve less than 0.1 milligrams of benzene per square inch at a temperature in excess of 430° F. Usually they evolve less than 0.04 milligrams of benzene per square inch at a temperature of at least 430° F. As shown in FIGS. 12 through 16, the containers of this invention comprise:

- (a) a sized paperboard blank having a basis weight suitable for a selected type of food container;
- (b) a base coat coating applied to one or both surfaces of the paperboard blank, the base coat coating comprising a mixture of an inorganic pigment and a polymer latex comprising aliphatic copolymers having the following monomers:



wherein R and R<sup>1</sup> may be the same or different aliphatic hydrocarbons having one to six carbon atoms and the ratio of (i) to (ii) is in the range of 1:100 to 100:1, preferably the range of (i) to (ii) is 1:3 to 3:1;

- (c) a top coat coating layer applied to the base coat coating layer, the top coat coating layer comprising an inorganic pigment and an aliphatic polymer latex comprising aliphatic copolymers having the following monomers:



wherein R and R<sup>1</sup> may be the same or different aliphatic hydrocarbons having 1 to 6 carbon atoms and the ratio of (i) to (ii) is in the range of 1:100 to 100:1, preferably 1:3 to 3:1.

In a preferred mode, both R and R<sup>1</sup> are methyl groups. The paperboard blank has suitably a weight in the range of about 100 to 400 lbs. per 3000 square foot ream and a caliper in the range of about 0.008 to 0.055 inches. In a suitable variant of this invention, sufficient moisture is introduced into the blank to produce a moisture content of about 4 to 12% by weight.

These microwaveable containers are suitably prepared by sizing a selected paperboard suitable for use as a food container by applying a base coating to one or both surfaces of the paperboard blank.

The base coat coating comprising a mixture of an inorganic pigment and a polymer latex comprising aliphatic copolymers having the following monomers:



wherein R and R<sup>1</sup> may be the same or different aliphatic hydrocarbons having one to six carbon atoms and the ratio of (i) to (ii) is in the range of 1:100 to 100:1;

A top coat coating layer applied to the base coat coating layer, the top coat coating layer comprising an inorganic pigment and an aliphatic polymer latex comprising aliphatic copolymers having the following monomers:



wherein R and R<sup>1</sup> may be the same or different aliphatic hydrocarbons having 1 to 6 carbon atoms and the ratio of (i) to (ii) is in the range of 1:100 to 100:1.

In a preferred embodiment, these paperboard containers include a microwave susceptible layer. This microwave susceptor layer is preferred for microwave cooking applications to give a brown appearance to cooked meat. Without the susceptor layer the food would also be cooked, but it would not have the pleasing brown color for meats preferred by consumers. At the microwave cooking temperatures, in excess of 430° F., it is essential that evolution of benzene be kept below 0.1 milligrams per square inch of the container surface, preferably below 0.04 milligrams per square inch of

(i)

(ii)

the container surface. In our process we can control the evolution of benzene to values below 0.03, 0.02, and 0.01 milligrams per square inch of the container. Usually benzene emission is increased when microwave susceptor layers are coated on the paperboard and/or the paperboard container. Metalized polyesters are suitably formed as a microwave susceptor layer on the paperboard surface as shown in FIG.

1. Aluminum and nickel are suitable metals.

In our process, the usual conventional papermaking fibers are suitable. We utilize softwood, hardwood, chemical pulp obtained from softwood and/or hardwood chips liberated into fiber by sulfate, sulfite, sulfide or other chemical pulping processes. Mechanical pulp was obtained by mechanical treatment of softwood and/or hardwood. Recycled fiber and other refined fiber may suitably be utilized in our paperboard manufacturing process.

Papermaking fibers used to form the paperboard used to form the microwaveable containers of this invention include cellulosic fibers commonly referred to as wood pulp fibers, liberated in the pulping process from softwood (gymnosperms or coniferous trees) and hardwoods (angiosperms or deciduous trees). The particular tree and pulping process used to liberate the tracheid are not critical to the success of the present invention. Cellulosic fibers from diverse material origins may be used to form the web of the present invention including cottonwood and non-woody fibers liberated from sabai grass, rice straw, banana leaves, paper mulberry (i.e., bast fiber), abaca leaves, pineapple leaves, esparto grass leaves, and fibers from the genus *Hesperaloe* in the family Agavaceae. Also recycled fibers which may contain any of the above fiber sources in different percentages can be used in the present invention.

Papermaking fibers can be liberated from their source material by any one of the number of chemical pulping processes familiar to one experienced in the art including sulfate, sulfite, polysulfite, soda pulping, etc. The pulp can be bleached if desired by chemical means including the use of chlorine, chlorine dioxide, oxygen, hydrogen peroxide, etc. Furthermore, papermaking fibers can be liberated from source material by any one of a number of mechanical/chemical pulping processes familiar to anyone experienced in the art including mechanical pulping, thermomechanical pulping, and chemi-thermomechanical pulping. These mechanical pulps can be bleached, if one wishes, by a number of familiar bleaching schemes including alkaline peroxide and ozone bleaching.

Generally in our process the range of hardwood to softwood varies from 0–100% to 100 to 0%. The preferred range for hardwood to softwood is about 20 to 80 to about 80 to 20; the most preferred range of hardwood comprises about 40 to about 80 percent of the furnish and the softwood comprises about 60 to about 20 percent of the furnish.

FIGS. 12, 13, 14, 15, and 16 provide a schematic layout of a suitable process for the manufacture of the useful paperboard and for the manufacture of the articles of manufacture of this invention useful in microwaving food and using the paperboard as raw material. These figures also show the microwave susceptor layer.

In FIG. 14 it is shown that feedstock is pumped into the mix box 40. Alum and other internal sizing agents are added to the feedstock along line 41 prior to it being pumped into the machine chest (44). Optionally a wet strength agent such as a Parez or Kymene is added to the feedstock through line (43) at the machine chest (44). Suitable wet strength agents are nitrogen containing polyamides. For food service products, if the food comes in contact with the wet strength agent, it has to be approved by the FDA Representative

polyamides are listed in European Patent Application 91850148.7 relating to polyamide epichlorohydrin (PAE) wet strength resins and that patent application is incorporated herein by reference. Parez 631NC which is a glyoxylated polyacrylamide is a suitable wet strength agent. In the stuff box (49) starch is charged through line (46), and optionally blue dye is charged through line (48); for pH control, a base such as caustic is charged through line (51). The cationic starch is added through line (54) and prior to the cleaners (55). The embryonic paperboard web is formed on the fourdrinier wire (58). The water is removed through a water removal apparatus (60). Initially the water is removed from the bottom side of the sheet through the fourdrinier table and from the top side of the web through the BelBond vacuum system. The web is heated with steam through steam showers (61), and the paperboard web is pressed in the press section (62) and dried in the dryer sections (63). Starch is supplied through line 64 to the size press (65). The web is passed through calender stacks (66) to smooth the web. Coating section (67) represents one to six coaters. The binder and optionally pigment is coated on both sides of the paperboard. Usually about three to six coatings are provided. For paper cup and related applications, usually the paperboard is not coated. The coated or uncoated paperboard is calendered in the gloss calender (68) and rolled on the reel (69). The paperboard is optionally placed in a printing press (70) for plate and bowl applications. Suitably a rotogravure press, flexopress or lithopress is utilized. Advantageously two to eight colors are printed on the reel. The printed reel is placed in a coater (71) where optionally two plate coatings are applied. Optionally, the reeled web is suitably moistened in a wetting applicator (72) (Dahlgren Press). The moistened web is wound onto a reel (73). A moistened web is utilized in the manufacture of articles which require significant deformation of the board. Representative articles requiring significant deformation of the board are bowls shown in FIGS. 1 and 2 and plates shown in FIG. 4. In FIG. 12 the paperboard manufacturing process is illustrated. In FIG. 16 at (80) the polyterephthalate film is applied to the paperboard where at (81) the surface is metalized, usually aluminized, at (82) the coated metalized surface is etched, at (83) adhesive is applied, at (84) we have the coated web which is shape cut at (85) and formed into containers such as bowls, and at (87) the bowls are stacked. Representative bowls made by the process set forth in FIG.

16 are shown in FIGS. 1 and 2.

Moisture may be introduced into the paperboard blank in the form of water or preferably as a moistening/lubricating solution. When blank stock in roll form is used, as in commercial scale operations, the blank stock is unrolled, coated as described above, wetted, rerolled, and allowed to stand for up to 24 hours or more before die-cutting is undertaken. Water is the preferred moistening solution.

In FIG. 15 the paperboard from reel (73) is fed into the die press (74) where the paperboard is scored and cut. This blank is fed into the die (75) which is capable of forming the desired articles of manufacture such as bowls, FIGS. 1 and 2; plates, FIG. 4; canisters, FIG. 3; French fry sleeves, FIG. 5; hamburger clam shells, FIG. 7; rectangular take-out containers, FIG. 6; food buckets, FIG. 10; cups, FIG. 8; food containers, FIG. 11; and other consumer products. Optionally these containers have a microwave susceptible layer to enable the browning of meat products.

The paperboard material is coated with a coating polymer which does not produce benzene when the container made from the paperboard is used in microwaving food prior to formation of the paperboard shells used in forming the

containers in accordance with the present invention. Polymers suitable for this purpose are aliphatic copolymers having the following monomers:



wherein R and R<sup>1</sup> may be the same or different aliphatic hydrocarbons having one to six carbon atoms and the ratio of (i) to (ii) is in the range of 1:100 to 100:1, preferably in the range of about 1:3 to 3:1.

Suitably a top coat coating layer is applied to the base coat coating layer, the top coat coating layer comprising an inorganic pigment and an aliphatic polymer latex comprising aliphatic copolymers having the following monomers:



wherein R and R<sup>1</sup> may be the same or different aliphatic hydrocarbons having 1 to 6 carbon atoms and the ratio of (i) to (ii) is in the range of 1:100 to 100:1, preferably in the range of 1:3 to 3:1.

The use of the above set forth coatings is expected to achieve a benzene evolution of less than 0.1 milligram per square inch of container surface at temperatures in excess of 430° F. Many manufacturers of microwaveable food products request that the benzene evolved at 430° F. be less than 0.04 milligrams per square inch of the container surface, sometimes less than 0.03 milligrams per square inch of container surface. In our process we can achieve a benzene evolution of less than 0.01 milligrams per square inch of the container surface.

Conveniently for microwave applications as shown in FIGS. 1 through 12, a microwave susceptor layer is laminated on top of the paperboard substrate on which a pigment has been coated. The microwave susceptor layer comprises alumina and polyester compositions. Polyethylene terephthalate is the preferred polyester composition, THERMXTM copolyester PCIA 6761 resin is also useful. The films in general are metalized polyesters wherein the metal is aluminum, nickel, etc.

The cooking of food and heating of substances with microwave radiation has become increasingly popular and important in recent years because of its speed, economy, and low power consumption. With food products, however, microwave heating has drawbacks. One of the major drawbacks is the inability to brown or sear the food product to make it similar in taste and appearance to conventionally cooked food.

One method involves the use of a metalized coating on paperboard. In this method, first, metal particles are vacuum deposited onto a film, preferably a polyester film. The film is then laminated onto the paper. The thus metalized paper, typically, must then be positioned onto a particular part of

the food package requiring a windowing operation. The windowing operation requires that the metallized paper be slit before entering the process.

A microwave interactive coating which is capable of being printed on a substrate is also suitable. This coating overcomes the problems inherent in vacuum deposited metal coatings because the coatings can be printed exactly where they are required. Furthermore, coating patterns, coating formulations, and coating thicknesses can all be varied using conventional printing processes. A printing process also allows the use of materials besides metals as microwave reactive materials, as well as providing the possibility for a wide range of heating temperatures and a wide variety of applications.

The microwave interactive printable coating composition comprises a microwave reactive material selected from a conductor or semiconductor, a dielectric, or a ferromagnetic and a binder.

The microwave interactive printable coating is coated onto a film which is further laminated to a microwave transparent substrate.

In another embodiment, a method of manufacturing a microwave interactive coated substrate is provided. This substrate comprises coating a substrate using a conventional printing process with a microwave interactive printable coating composition comprising a microwave reactive material selected from a conductor or semiconductor, a dielectric, or a ferromagnetic, and a binder.

Microwave reactive materials (MRM) are capable of converting microwave energy to heat. This is accomplished using either the conductive or semiconductive properties, dielectric properties, or ferromagnetic properties of the microwave reactive materials. The materials having these properties will hereafter be referred to as conductors, semiconductors, dielectrics or ferromagnetics.

The microwave reactive materials included within the scope of this invention include any material which has suitable conductive or semiconductive, dielectric or ferromagnetic properties so that the material is capable of converting microwave radiation to heat energy. The materials can have any one of the above properties or can have a combination of the above properties. Furthermore, the properties of the substrate on which the material is coated, such as the orientation, heatset temperature, and melting point, as well as the adhesion between the coating and the substrate will affect the reactivity of the materials to microwave energy.

The type and amount of microwave reactive materials used in the coating composition generally determines the degree of interaction with the microwaves and hence the amount of heating. In a preferred embodiment where the material used is conductive, the amount of heat generated is a function of the product of the conductivity of the material and the thickness of the material. In one aspect of this embodiment, when the microwave reactive material is carbon, the microwave reactive material combined with binder will preferably have a resistivity ranging from 50 ohms per square to 10,100 ohms per square. Our containers containing a microwave susceptible layer cannot evolve more than 0.1 milligram of benzene per square inch of container surface. Preferably no more than 0.04 milligrams of benzene are evolved and most preferably less than 0.03 milligrams of benzene are evolved. This low benzene evolution has to be maintained at cooking temperatures of 430° F. or more.

Generally any metal, alloy, oxide, or any ferrite material which has microwave reactive properties as described above

can be used as a microwave reactive material. Microwave reactive materials include suitable compositions comprising aluminum, iron, nickel, copper, silver, carbon, stainless steel, nichrome, magnetite, zinc, tin, iron, tungsten, titanium, and the like. The materials can be used in a powder form, flake form, or any other finely divided form which can be suitably used in printing processes. The microwave reactive materials can be used individually or can be used in combination with other microwave reactive materials.

In the preferred embodiment, the microwave reactive material will be suitable for food packaging. Alternatively, the microwave reactive material will be separated from the food by a film or other protective means.

It is preferred that the microwaver reactive materials demonstrate rapid heating to a desired temperature, with subsequent leveling off of the temperature, without arcing during the material's exposure to microwave radiation. The temperature at which the microwave reactive material levels off is hereinafter referred to as the operating temperature. Generally the microwave reactive material will operate at a temperature ranging from about 430° F. to 480° F.

The microwave reactive material is combined with a binder to form a coating composition. The binder used in this invention can comprise any aqueous or hydrocarbon dispersed or dissolved material that can be used in a printing process provided it does not evolve more than 0.1 milligrams of benzene per square inch, preferably less than 0.04 milligrams, and most preferably less than 0.03 milligrams of benzene per square inch. Suitable binders are aliphatic copolymers having the following monomers:



wherein R and R<sup>1</sup> may be the same or different aliphatic hydrocarbons having one to six carbon atoms and the ratio of (i) to (ii) is in the range of 1:100 to 100:1, preferably 1:3 to 3:1.

The binder must have good thermal resistance and suffer little or no degradation at the temperatures generated by the microwave reactive material. It must also have an adhesive ability which will allow it to adhere to the substrate.

In one preferred embodiment of this invention, an important aspect is that the microwave reactive material coated substrate must shrink during the heating process at a controlled rate so that the temperature of the coating rises rapidly and then remains at a constant level. In this embodiment it is important that the binders chosen be adhesive enough to bind the microwave reactive material to the substrate during the treatment with microwave energy.

The binder and the microwave reactive material are generally combined in a suitable ratio such that the microwave reactive material, in the form of a thin film, can convert the microwave radiation to heat to raise the temperature of a food item placed thereon, yet still have sufficient binder to be printable and to adhere to the film. There should also be sufficient binder present to prevent arcing of the microwave reactive material.

Generally the ratio of the microwave reactive material to binder, on a solids basis, will depend upon the microwave reactive material and binder chosen. In a preferred embodi-

ment where the microwave reactive material is nickel, the microwave reactive material to binder ratio, on a weight basis, should be about 2:1 or higher.

Other materials can be included in the coating composition such as surfactants, dispersion aids, and other conventional additives for printing compositions. The coating can be applied using conventional printing processes such as rotogravure, flexography, and lithography. After the coating composition has been applied, it can be dried using conventional printing ovens normally provided in a printing process.

Generally, any amount of coating can be used. The amount of heat generated will vary according to the amount and type of coating applied to the substrate. In a suitable embodiment, when the coating material is nickel, the amount of coating will range from about 3 to about 11 pounds per 3000 square foot ream.

The coating composition can generally be coated upon any substrate such as paper or paperboard or any suitable film material which does not melt at temperatures of about 430° F. to 500° F. and does not evolve more than 0.04 milligrams of benzene per square inch of surface at these temperatures.

A desirable feature for the microwave reactive coated substrates is that the substrate should either shrink during the heating process at a controlled rate or in some other manner the interparticle network of the coating should be disrupted so that the temperature of the coating rises rapidly and then remains at a constant level.

In a preferred embodiment of this invention, the coating composition is printed onto an oriented film. The film can be selected from any known films such as polyesters, nylons, polycarbonates, and the like. The film used generally should be shrinkable at the operating temperatures of the microwave reactive material but any film material which shrinks can be used. The film must also have a melting point above the operating temperature of the microwave reactive material. That is, it must melt above 430° F. to 500° F. and evolve no more than 0.04 milligrams of benzene per square inch of the container surface at a temperature of at least 430° F. A particularly preferred class of films include oriented polyester films such as Mylar®.

The thus coated film is then applied to a microwave transparent substrate. The substrate, preferably, is also dimensionally stable at the operating temperature of the microwave reactive material. Typical substrates include paper and paperboard.

The film is attached to the substrate using conventional adhesives. The adhesives used must be able to withstand heating temperatures within the operating range of the microwave reactive material that is a temperature of about 430° F. to 480° F. The adhesive must also be able to control the rate at which the film shrinks and must not evolve benzene more than 0.03 milligrams per square inch of the paperboard container surface.

Suitable microwaveable packages comprise a dielectric substrate substantially transparent to microwave radiation having at least a portion of at least one surface thereof coated with a coating composition comprising a dielectric polymeric matrix having incorporated therein (a) particles of a microwave susceptor material; and (B) particles of a blocking agent.

In general, the dielectric substrate may be any material having sufficient thermal and dimensional stability to be useful as a packaging material at the high temperatures which may be desired for browning or rapidly heating foods in a microwave oven (e.g., at temperatures in excess of 430°

F.). Useful substrates include polymeric terephthalate films as well as polymethylpentene films and films of other thermally stable polymers such as polyacrylates, polyamides, polycarbonates, polyetherimides, polyimides, and the like, provided they do not evolve more than 0.04 milligrams of benzene per square inch of the container surface at temperatures in excess of 430° F. Moreover, porous structures such as paper or non-woven materials can also be employed as substrates so long as the required thermal and dimensional stability is satisfied. For flexible packaging the substrate is preferably about 8 to 50 micrometers thick. Thicker, non-flexible materials, such as found in trays, lidding, bowls, and the like, may also be employed.

Suitably, the substrate must have sufficient dimensional stability at the elevated temperatures (430° F. to 480° F.) involved in microwave cooking to prevent distortion of the substrate which may result in non-uniform cooking from loss of intimate contact of the packaging material with the food to be cooked. Substrates normally lacking such high temperature dimensional stability can be used if they are laminated with yet another substrate layer meeting the thermal stability requirements of the original substrate and do not evolve benzene more than 0.03 milligrams per square inch of the paperboard container surface. The lamination can be accomplished either by taking advantage of the adhesive properties of the thermoplastic matrix coating on the original substrate or by using any number of conventional adhesives to aid in forming a stable laminate. For example, a polyester copolymer coated polyethylene terephthalate film can be thermally sealed to another polyester film or to paper or heavier ovenable paperboard. Alternatively, another adhesive can be applied from solution prior to lamination to increase the strength of the laminate. These supplemental adhesives can be selected from a number of commercially available candidates with required thermal stability. These include copolymers, copolyester-polyurethanes, and cyanoacrylates.

The dielectric polymeric material forming the matrix of the coating composition may be composed of a variety of materials which, when deposited onto a suitable substrate, exhibit sufficient thermal stability to allow for dimensional integrity of the final packaging material at the elevated temperatures (430° F. to 480° F.) associated with microwave cooking of food.

The dielectrical properties at 915 megahertz and 2450 megahertz of the matrix formed by the deposition of the polymeric material upon the packaging substrate is an important variable in terms of the heat generated in unit time at 2450 Mhz. Specifically, the dielectric matrix should, in general, possess a relative dielectric constant of between about 2.0 and about 10, preferably of between about 2.1 and about 5, and should generally possess a relative dielectric loss index of between about 0.001 and about 2.5, preferably of between about 0.01 to 0.6. The matrix also preferably displays adhesive characteristics to the substrate as well as to any additional substrate to which the composite may be laminated to increase dimensional stability.

The microwave susceptor materials employed include any materials which are capable of absorbing the electric or magnetic portion of the microwave field energy and converting that energy into heat. Suitable materials include metals such as powdered nickel, antimony, copper, molybdenum, bronze, iron, chromium, tin, zinc, silver, gold, and aluminum. Other conductive materials such as graphite and semi-conductive materials such as silicon carbides and magnetic material such as metal oxides (if available in particulate form) may also be utilized. Particularly preferred

susceptor materials include alloys of copper, zinc, and nickel sold under the designation SF401 by Oboron; as well as leafing aluminum powder.

Suitable susceptor materials employed are in particulate form. Such particles may be flakes or powders. The size of such particles will vary in accordance with a number of factors, including the particular susceptor material selected, the amount of heat to be generated, the manner in which the coating composition is to be applied, and the like.

Typically, however, when such coating compositions are to be applied in the form of inks, due to limitations of the printing processes, such powders will have diameters of no more than about 50 microns. In general, in such circumstances, particle sizes of between about 0.1 and about 25 microns are preferably employed. When the susceptor materials are employed in the form of flakes (e.g., such as in the form of leafing aluminum), such flakes are typically of those sizes of flakes routinely used in the gravure ink art for the printing of metallic coatings.

A suitable blocking agent employed comprises at least one member of the group consisting of calcium salts, zinc salts, zinc oxide, lithopone, silica, and titanium dioxide. Preferred blocking agents include calcium carbonate, calcium sulfate, zinc oxide, silica, and titanium dioxide, and calcium carbonate, with calcium carbonate being most preferred.

Suitable blocking agents are typically employed in particulate form. The particle size of such blocking agents is generally limited by the particular coating process employed, and when such coating is applied in the form of an ink, such particle size is typically less than about 50 microns, with particle sizes of between about 0.1 and about 25 microns being preferred for most blocking agents. When calcium carbonate is employed as the blocking agent, particle sizes of between about 1 and about 10 microns are more preferred, with particle sizes of between 3 and about 7 microns being most preferred.

It is believed that the presence of such blocking agents control the amount of heat generated by the susceptor material. By controlling the ratio and amount of blocking agent and susceptor, and/or by varying the thickness of the ink applied, the amount of heat generated by a preselected dosage of microwave radiation may be consistently controlled within a preselected range. In applications contemplated by this invention, the temperature will be in excess of 430° F.

Variables which must be taken into account for determining the precise ratios of susceptor to blocking agent needed for any particular use include the physical size, shape, and surface characteristics of the susceptor and blocking agent particles contained in the coating composition, the amount of coating composition to be applied to the substrate, and the portion size as well as the food to be cooked in such application. By so altering these variables as well as the susceptor:blocking agent ratio employed, one of ordinary skill can easily regulate the compositions utilized herein to heat to high temperatures in a controlled manner in relatively short periods of time in conventional microwave ovens, e.g., to temperatures above 430° F. in 120 seconds when subjected to microwave energy generated in dosages typically produced by such ovens, e.g., at 550 watts at 2450 megahertz.

The susceptor level in the matrix will generally range from about 3 to about 80% by weight of the combined susceptor blocking agent/matrix composition. As noted above, the optimum levels of susceptor material and of blocking agent incorporated into the coating compositions

will depend upon a number of factors, depending upon the ultimate end use employed. However, it has been found that, in many instances, weight ratio of 1:4 or more of blocking agent susceptor material will effectively prevent heating of the coating composition when subjected to dosages of microwave radiation generated by conventional microwave ovens. Lower ratios of blocking agent to receptor material will result in higher temperatures.

One of ordinary skill in the art can easily determine optimum ratios for any particular application using routine experimentation.

In addition to the blocking agent, polymeric material liquid carrier and susceptor material the coating composition employed in the microwavable package may optionally contain other conventional additives such as surface modifiers such as waxes and silicones, antifoam agents leveling agents, surfactants, colorants such as dyes and pigments and the like, which additives are well known to those of ordinary skill in the art.

Suitable microwavable packaging ink composition comprises a liquid carrier having dispersed or dissolved therein (A) a matrix-forming dielectric polymeric material substantially transparent to microwave radiation; (B) particles of a susceptor material; and (C) particles of a blocking agent.

The liquid carriers which may be employed include those organic solvents conventionally employed in the manufacture of ink as well as water and mixtures of one or more of the foregoing. Illustrative of such solvents are liquid acetates such as isopropyl acetate and the like; alcohols such as isopropanol, butanol, and the like; ketones such as methyl ethyl ketone and the like. Particularly preferred solvents include water, isopropyl acetate, and mixtures of isopropyl acetate. These solvents cannot evolve more than 0.03 milligrams of benzene per square inch of container surface at a temperature of 430° F.

The coating formulation may also include a mineral filler to increase the solids level of the polymeric binder mixture. The mineral filler should be present at a level of about 0 to 50 percent by weight and more preferably about 20 to 40 percent by weight. Suitable mineral fillers include, for example, kaolin clays, calcium carbonate, titanium dioxide, zinc oxide, chalk barite, silica, talc, bentonite, glass powder, alumina, graphite, carbon black, zinc sulfide, alumina silica, and mixtures thereof. Hydrafine clay, which is a hydrated aluminum silicate or kaolin with 0.9–2.5% titanium dioxide manufactured by J.M. Huber Corp. of Macon, Ga. is one preferred mineral filler.

By way of example, suitable surface sizing agents include starch, starch latex copolymers, animal glue, methyl cellulose, carboxymethyl cellulose, polyvinyl alcohol, and wax emulsions. Preferably, starch or a starch latex copolymer is employed as a sizing agent. By way of example, suitable commercially available sizing agents containing starch include "PENFORD® GUMS 200," "PENFORD® GUMS 220," "PENFORD® GUMS 230," "PENFORD® GUMS 240," "PENFORD® GUMS 250," "PENFORD® GUMS 260," "PENFORD® GUMS 270," "PENFORD® GUMS 280," "PENFORD® GUMS 290," "PENFORD® GUMS 295," "PENFORD® GUMS 300," "PENFORD® GUMS 330," "PENFORD® GUMS 360," "PENFORD® GUMS 380," "PENFORD® GUMS PENCOTE®," "PENFORD® GUMS PENSURF," "PENGLOSS®," "APOLLO® 500," "APOLLO® 600," "APOLLO® 600-A," "APOLLO® 700," "APOLLO® 4250," "APOLLO® 4260," "APOLLO® 4280," "ASTRO® GUMS 3010," "ASTRO® GUMS 3020," "ASTROCOTE® 75," "POLARIS® GUMS

LV," "ASTRO®×50," "ASTRO®×100," "ASTRO®×101," "ASTRO®×200," "ASTRO® GUM 21," "CALENDER SIZE 2283," "DOUGLAS®-COOKER 3006," "DOUGLAS®-COOKER 3007," "DOUGLAS®-COOKER 3012-T," "DOUGLAS®-COOKER 3018," "DOUGLAS®-COOKER 3019," "DOUGLAS®-COOKER 3040," "CLEARSONG GUMS 7," "CLEARSONG GUMS 8," "CLEARSONG GUMS 9," "CLEARSONG GUMS 10," "DOUGLAS®-ENZYME 3622," "DOUGLAS®-ENZYME E-3610," "DOUGLAS®-ENZYME E-3615," "DOUGLAS®-ENZYME 3022," "DOUGLAS®-ENZYME 3023," "DOUGLAS®-ENZYME 3024," "DOUGLAS®-ENZYME E," "DOUGLAS®-ENZYME EC," "CROWN THIN BOILING X-10," "CROWN THIN BOILING X-18," "CROWN THIN BOILING XD," "CROWN THIN BOILING XF," "CROWN THIN BOILING XH," "CROWN THIN BOILING XJ," "CROWN THIN BOILING XL," "CROWN THIN BOILING XN," "CROWN THIN BOILING XP," "CROWN THIN BOILING XR," "DOUGLAS®-UNMODIFIED PEARL," and "DOUGLAS®-UNMODIFIED 1200." These sizing agents are all commercially available from Penford Products Co. "PENFORD®," "PENCOTE®," "PENSRAE®," "PENGLOSS®," "APOLLO®," "ASTRO®," "ASTROCOTE®," "POLARIS®," "DOUGLAS®," and "CLEARSONG®" are all registered trademarks of Penford Products Co. Other suitable starches, including "SILVER MEDAL PEARL™," "PEARL B," "ENZO 32 D," ENZO 36W," ENZO 37D," SUPERFILM 245D," "SUPERFILM 270W," "SUPERFILM 240DW," "SUPERFILM 245D," SUPERFILM 270W," "SUPERFILM 280DW," "PERFORMER 1," "PERFORMER 2," "PERFORMER 3," "CALIBER 100," "CALIBER 110," "CALIBER 124," "CALIBER 130," "CALIBER 140," "CALIBER 150," "CALIBER 160," "CALIBER 170," "CHARGE +2," "CHARGE +4," "CHARGE +7," "CHARGE +9," "CHARGE +88," "CHARGE +99," "CHARGE +110," "FILMFLEX 40," "FILMFLEX 50," "FILMFLEX 60," and "FILMFLEX 70" are all commercially available from Cargill, Inc.

The cationic wet strength agent used in the manufacture of the paperboard can be selected from among those cationic wet strength agents known in the art such as dialdehyde starch, polyethylenimine, mannogalactan gum, glyoxal, and dialdehyde mannogalactan. A particularly useful class of wet strength agent is cationic glyoxylated vinylamide wet strength resins.

Glyoxylated vinylamide wet strength resins useful herein are described in U.S. Pat. No. 3,556,932 to Coscia. These resins are typically reaction products of glyoxal and pre-formed water soluble vinylamide polymers. Suitable poly-vinylamides include those produced by copolymerizing a vinylamide and a cationic monomer such as 2-vinylpyridine, 2-vinyl-N-methylpyridinium chloride, diallyldimethyl ammonium chloride, etc. Reaction products of acrylamide diallyldimethyl ammonium chloride in a molar ratio of 99:1 to 75:25 glyoxal, and polymers of methacrylamide and 2-methyl-5-vinylpyridine in a molar ratio of 99:1 to 50:50, and reaction products of glyoxal and polymers of vinyl acetate, acrylamide and diallyldimethyl ammonium chloride in a molar ratio of 8:40:2 are more specific examples provided by Coscia. These vinylamide polymers may have a molecular weight up to 1,000,000, but polymers having molecular weights less than 25,000 are preferred. The vinylamide polymers are reacted with sufficient glyoxal to provide a water soluble thermoset resin. In most cases the molar ratio of glyoxal derived substituents to amide substituents in

the resin is at least 0.06:1 and most typically 0.1:1 to 0.2:1. A commercially available resin useful herein is Perez 631 NC sold by Cytec Industries.

The cationic wet strength agent is generally added to the paperboard web in an amount up to about 8 pounds per ton or 0.4 wt %. Generally, the cationic wet strength agent is provided by the manufacturer as an aqueous solution and is added to the pulp in an amount of about 0.05 to 0.4 wt % and more typically in an amount of about 0.1 to 0.2 wt %. Unless otherwise indicated, all weights and weight percentages are indicated herein on a dry basis. Depending on the nature of the resin, the pH of the pulp is adjusted prior to adding the resin. The manufacturer of the resin will usually recommend a pH range for use with the resin. The Perez 631NC resin can be used at a pH of about 4 to 8.

Other wet strength agents used in preparing the paperboards having a low benzene evolution at microwave conditions of this invention can be selected from among those aminoplast resins (e.g., urea-formaldehyde and melamine-formaldehyde) resins and those polyamine-epichlorohydrin, polyamine epichlorohydrin or polyamide-amine epichlorohydrin or polyamide-amine epichlorohydrin resins (collectively "PAE resins") conventionally used in the papermaking art. Representative examples of these resins are described throughout the literature. See, for example, *Wet Strength in Paper and Paperboard*, TAPPI Monograph Series No. 29, TAPPI Press (1952) John P. Weidner, Editor, Chapters 1, 2 and 3 and U.S. Pat. Nos. 2,345,543 (1944); 2,926,116 (1965); and 2,926,154 (1960). Typical examples of some commercially available resins include the PAE resins sold by Hercules under the name Kymene, e.g., Kymene 557H and by Georgia Pacific under the name Amres, e.g., Amres 8855.

Kymene type wet strength agent is added to the paper fiber in an amount up to about 8 pounds per ton or 0.4 wt % and typically about 0.01 to 0.2 wt % and still more typically about 1 to 2 pounds per ton or 0.5 to 0.1 wt %. The exact amount will depend on the nature of the fibers and the amount of wet strength required in the product. These resins are generally recommended for use within a predetermined pH range which will vary depending upon the nature of the resin. For example, the Amres resins are typically used at a pH of about 4.5 to 9. It should be understood that since the use of the paperboard of the invention having low benzene evolution will be used to make articles used in connection with food service, all the wet strength additives used to make articles for food service products should have FDA approval if the wet strength agents come into direct contact with the food products.

The binder used in the manufacture of the paperboard, optionally in conjunction with the pigment, is applied in the coating section. The aliphatic polymeric binder has been described herein above; and under microwave use conditions, e.g., at temperatures in excess of 430° F. evolves less than 0.04 milligrams of benzene per one square inch of the board coating surface. Advantageously the clay pigment may be any suitable clay known to the art. For example, suitable pigments include kaolin clay, engineered clays, delaminated clays, structured clays, calcined clays, alumina, silica, aluminosilicates, talc, zinc sulfide, bentonite, glass powder, calcium sulfate, ground calcium carbonates, precipitated calcium carbonates, barite, titanium dioxide, and hollow glass or organic spheres. These pigments may be used individually or in combination with other pigments. Preferably the clay is selected from the group consisting of kaolin clay and conventional delaminated pigment clay. A commercially available delaminated pigment clay is

"HYDRAPRINT" slurry, supplied as a dispersion with a slurry solids content of about 68%. "HYDRAPRINT" is a trademark of Huber.

The pigment composition may also comprise other additives that are well known in the art to enhance the properties of coating compositions or are well known in the art to aid in the manufacturing process. For example, suitable additives include defoamers, antifoamers, dispersants, lubricants, film-formers, crosslinkers, thickeners and insolubilizers.

A suitable defoamer includes "Foamaster DF122NS" and "Foamaster VF." "Foamaster DF122NS" is a trademark of Henkel.

A suitable organic dispersant includes "DISPEX N-40" comprising a 40% solids dispersion of sodium polycarboxylate, "DISPEX N-40" is a trademark of Allied Colloids and Berchem® 4290; a complex organic dispersant; and Berchem® 4809, a polyacrylate dispersant supplied by Berchem Inc. Other suitable dispersants are Accumer® 9000 and Accumer® 9500, polyacrylate dispersants; Tamol® 731; Tamol® 850, a sodium salt of polymeric carboxylic acid; Tamol® 960, a sodium salt of a carboxylated acrylic polyelectrolyte; and Tamol® 983, an organic polyacid dispersant. The Tamol dispersants are supplied by the Rohm & Haas Company. Polyphosphates and hexametaphosphates are also suitable dispersants.

A suitable coating lubricant includes "BERCHEM 4095" which is a 100% active coating lubricant based on modified glycerides. "BERCHEM 4095" is a trademark of Berchem. Other suitable lubricants are Berchem® 4000, a polyethylene emulsion; Berchem® 4060, a polyethylene emulsion; Berchem® 4110; Berchem® 4113, a modified diglyceride; Berchem® 4300, a fatty acid dispersion; Berchem® 4320, a fatty acid dispersion; and Berchem® 4569, a diglyceride emulsion, all supplied by Berchem Inc. In addition, the following lubricants are utilized: HTI Lubricant 1000, calcium stearate; HTI Lubricant 1100, a calcium stearate/polyethylene co-emulsion; and HTI Lubricant 1050, a polyethylene/carnauba wax co-emulsion supplied by Hopton Technologies, Inc.; and Sunkote® 455, calcium stearate supplied by Sequa Chemicals, Inc.

Suitable thickeners including the sodium alginate moiety are: Kelgin® LV, Kelgin® XL, Kelgin® RL, and Keigin® QL; SCOGIN™ QH, SCOGIN™ LV, and SCOGIN™ QL. Other suitable thickeners are propylene glycol alginates such as Kelcolloid® LVF; treated sodium alginates such as Kelgin® QM and Kelgin® QL. The Kelgin products are supplied by Merck & Co., Inc., and the Scogin products are supplied by Pronova Biopolymer, Inc.

The deposition of the mixture onto the wire may be referred to as web laydown and an embryonic paper web is formed thereby. The embryonic web comes off the screen and is carried on various fabrics or felts where it undergoes wet pressing by suitable papermaking apparatus known in the art. After wet pressing, the embryonic web is about 60% water and about 40% papermaking fiber and other solid material discussed previously.

The embryonic web then undergoes further drying processes, such as by means of vacuum boxes, through-air dryers, steam heated dryers, gas-fired dryers, or other suitable methods.

The paperboard useful for the manufacture of microwaveable containers of this invention can advantageously be produced under acid, alkaline or neutral sizing conditions. Suitable internal sizing agents include rosin and alum, waxes, fatty acid derivatives, hydrocarbon resins, alkyl ketene dimers, and alkenyl succinic anhydrides. Alkenyl

succinic anhydrides are organic chemicals comprising an unsaturated hydrocarbon chain containing pendant succinic anhydride moiety. Monocarboxylic fatty acids having a chain length of C<sub>8</sub> to C<sub>22</sub> are also suitable internal sizing agents. The rosin sizing agents include gum rosin, wood rosin, and tall oil rosin. Suitable C<sub>8</sub> to C<sub>22</sub> fatty acids useful as internal sizing agents include copyrylic, capric, lauric, myristic, palmitic, stearic, arachidic, betenic, palmitoleic, oleic, ricinoleic, petroselinic, vaccenic, linoleic, linolenic, eleostearic, licenic, paranirac, gadoleic, arachidonic, cetoleic, and erycic.

Alum or aluminum salts used to prepare suitable paperboards useful for the manufacture of microwaveable containers of this invention are water-soluble, and they may be aluminum sulfate, aluminum chloride, aluminum nitrate, or acid aluminum hydrophosphates in which P:Al=1.1:1-3:1.

When aluminum salts or their mixtures are used, a base is added to form aluminum hydroxide having anionic surface charges. The base used is suitably sodium or potassium hydroxide, sodium or potassium carbonate, sodium or potassium metasilicate, sodium or potassium watergasses, sodium or potassium phosphate or borate, or sodium or potassium aluminate, or mixtures of these.

Aluminate compounds such as sodium aluminate or potassium aluminate are also used as the water-soluble aluminum salts. In this case, acid is added in order to form, within the pH range 7-9, an aluminum hydroxide having anionic surface charges. The acid used is a mineral acid such as sulfuric acid, hydrochloric acid, nitric acid or phosphoric acid, or organic acids such as oxalic acid, citric acid or tartaric acid. Suitably the acids used may also be acid aluminum salts such as aluminum sulfate, aluminum chloride, aluminum nitrate, or various water-soluble aluminum hydrophosphates.

Suitably water-soluble polymeric aluminum salts, i.e., polyaluminum salts, so-called basic aluminum salts, which are also called polyaluminum hydroxy salts or aluminum hydroxy salts are also used. In addition, the following salts are utilized: polyaluminum sulfate, polyaluminum chloride and polyaluminum chloride sulfate. The polyaluminum salt does suitably, in addition to the chloride and/or sulfate ion, also contain other anions, e.g., phosphate, polyphosphate, silicate, citrate, oxalate, or several of these.

Commercially available polymeric aluminum salts of this type include PAC (polyaluminum chloride), PAS (polyaluminum sulfate), UPAX 6 (silicate-containing polyaluminum chloride), and PASS (polyaluminum sulfate silicate).

The net formula of the water-soluble polyaluminum salt may be, for example:



and its alkalinity may vary so that the m-value ranges from 1 to 5 (alkalinity is respectively 16-83% according to the formula (m:6)×100). In this case the ratio Al/OH is 2:1-1:2.5. n is 2 or higher.

When a polyaluminum compound is used, it may be desirable to add a base in order to optimize the Al/OH ratio, even if all of the polyaluminum compounds in accordance with the invention do work as such.

The base or acid which forms in situ an aluminum hydroxide with the aluminum salt may be added to the fiber suspension, or just before the aluminum salt, or after it, or simultaneously with it.

The aluminum hydroxide may also be formed before the moment of addition, for example in the adding tube, or in advance in sol form.

The amount of the aluminum salt, calculated as  $\text{Al}_2\text{O}_3$ , is preferably approximately 0.01–1.0% of the dry weight of the pulp.

The following examples are intended to be illustrative of the present invention and to teach one of ordinary skill how to make use of the invention. These examples are not intended to limit the invention or its protection in any way.

### EXAMPLES

Usually two coatings are applied to the wire side of the paperboard by the use of in-line blade coaters. The coated surface is then printed by conventional printing techniques. The microwave susceptor is then applied to the coated surface in a separate converting operation. These processes are set forth in FIGS. 15 and 16, numbers (70) to (87).

In one embodiment, only one side of the paperboard is coated. The coated side has coating No. 2 (described in Table 2) immediately adjacent the paperboard basestock. Coating No. 3 (described in Table 3) is applied on top of coating No. 2. The microwave susceptor is then applied to the top surface.

Alternatively, coating No. 1 (described in Table 1) is applied to one surface of the paperboard and coatings No. 2 and 3 are applied to the other surface. In this case the microwave susceptor is applied to either side of the coated surface.

TABLE 1

| Composition of Coating No. 1 |       |
|------------------------------|-------|
| Material                     | Parts |
| No. 1 Clay                   | 100.0 |
| Latex                        | 20.0  |
| Thickener                    | 0.5   |
| Ammonia                      | 0.3   |
| Dispersant                   | 0.1   |

TABLE 2

| Composition of Coating No. 2 |       |
|------------------------------|-------|
| Material                     | Parts |
| No. 2 Clay                   | 90.0  |
| Calcium carbonate            | 10.0  |
| Latex                        | 19.3  |
| Thickener                    | 0.1   |
| Ammonia                      | 0.1   |
| Dispersant                   | 0.1   |

In both tables, the latexes were Rohm & Haas EXP 3368, Rohm and Haas Polyco 3103, BASF Acronal S-504, and Experimental latex from GenCorp. Rohm & Haas EXP 3368 is a copolymer that consists of 69% by weight poly(vinyl acetate) and 31% by weight poly(butyl acrylate) based on the quantitative carbon-13 NMR analysis. No other co-monomers were detected in this resin by C-13 NMR.

Table 3 shows that only the Rohm & Haas EXP 3368 and Rohm & Haas Polyco 3103 evolved less than 0.04 milligrams of benzene per square inch of board or container surface at a temperature in excess of 430° F.

TABLE 3

| Composition of Coating No. 3                                 |             |
|--------------------------------------------------------------|-------------|
| Benzene evolved at 430° F. $\mu\text{g}/\text{in.}^2$        |             |
| Styrene-butadiene                                            | 0.700       |
| Experimental latex from GenCorp                              | 0.180       |
| Styrene-acrylic-acrylonitrile copolymer (BASF Acronal S 504) | 0.011–0.020 |
| Rohm & Haas EXP 3368                                         | 0.010       |
| Rohm & Haas Polyco 3103                                      |             |

Using the alternate method where one side is coated with coatings 2 and 3 and the other side is coated with coating 1 produced the results shown in Table 4. The latex used in Table 4 was Rohm & Haas EXP 3368.

TABLE 4

| Reel No.              | Coat Weight (#/3000 ft <sup>2</sup> ) T.S. | Coat Weight (#/3000 ft <sup>2</sup> ) W.S. | Benzene milligrams/in. <sup>2</sup> |
|-----------------------|--------------------------------------------|--------------------------------------------|-------------------------------------|
| 2242<br>(16 pt board) | 13.8                                       | 4.3                                        | 0.0094                              |
| 2243<br>(16 pt board) | 14.6                                       | 3.8                                        | 0.0070                              |
| 2244<br>(18 pt board) | 7.5                                        | 3.6                                        | 0.0087                              |

W.S. = Wire Side; T.S. = Top Side of the board

I claim:

1. A microwaveable, food contact compatible, disposable, rigid and strong paperboard useful as a base stock for forming substantially high microwaveable food containers comprising:

(a) a sized paperboard blank having a basis weight suitable for a food container;  
 (b) a base coat coating applied to one or both surfaces of the paperboard blank, the base coat coating comprising a mixture of an inorganic pigment and an acrylic latex comprising aliphatic copolymers having the following monomers:



(i)

(ii)

wherein R and  $\text{R}^1$  may be the same or different aliphatic hydrocarbons having one to six carbon atoms and the ratio of (i) to (ii) is in the range of 1:100 to 100:1;

(c) a top coat coating layer applied to the base coat coating layer, the top coat coating layer comprising an inorganic pigment and an aliphatic polymer latex comprising aliphatic copolymers having the following monomers:



(i)

-continued



wherein R and R<sup>1</sup> may be the same or different aliphatic hydrocarbons having one to six carbon atoms and the ratio of (i) to (ii) is in the range of 1:100 to 100:1; and wherein said coated microwaveable paper board evolves less than 0.1 milligrams of benzene per square inch of the paperboard surface at temperatures in excess of 430° F. while exposed to microwave.

2. The paperboard of claim 1 wherein R and R<sup>1</sup> are —CH<sub>3</sub> groups and the paperboard evolves less than 0.04 milligrams of benzene per square inch of the paperboard surface at a temperature in excess of 430° F.

3. The paperboard of claim 1 or claim 2 wherein the base coat and the top coat are copolymer latex comprising comonomers of vinylacetate and butylacrylate.

4. The paperboard of claim 1 or claim 2 wherein the base coat and top coat are copolymer latex comprising comonomers of vinylacetate and acrylate.

5. The cellulosic paperboard of claim 1 or claim 2 wherein the paperboard is coated on one side with a metalized polyester to provide a food container with a microwave susceptor layer.

6. The cellulosic paperboard of claim 5 wherein the metal is aluminum.

7. The cellulosic paperboard of claim 5 wherein the metal is nickel.

8. The cellulosic paperboard of claim 5 wherein the metal coating is selected from the group consisting of aluminum, iron, nickel, copper, silver, carbon, stainless steel, nichrome, magnetite, zinc, tin, tungsten, titanium, and mixtures of these.

9. A microwaveable, food contact compatible, disposable, rigid and strong paperboard container comprising:

- (a) a sized paperboard blank having a basis weight suitable for a food container;
- (b) a base coat coating applied to one or both surfaces of the paperboard blank, the base coat coating comprising a mixture of an inorganic pigment and an acrylic latex comprising aliphatic copolymers having the following monomers:



wherein R and R<sup>1</sup> may be the same or different aliphatic hydrocarbons having one to six carbon atoms and the ratio of (i) to (ii) is in the range of 1:100 to 100:1;

- (c) a top coat coating layer applied to the base coat coating layer, the top coat coating layer comprising an inorganic pigment and an aliphatic polymer latex comprising aliphatic copolymers having the following monomers:

(ii)



(i)

(ii)

5

wherein R and R<sup>1</sup> may be the same or different aliphatic hydrocarbons having one to six carbon atoms and the ratio of (i) to (ii) is in the range of 1:100 to 100:1; and wherein said coated rigid microwaveable food container evolves less than 0.1 milligrams of benzene per square inch of the container surface at temperatures in excess of 430° F. while exposed to microwave.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9

26. The microwaveable container of claim 15 in the form of a canister.

27. The microwaveable container of claim 18 in the form of a canister.

28. The microwaveable container of claim 15 in the form of a rectangular take-out container.

29. A process for producing substantially rigid, microwaveable food containers from a coated paperboard comprising the steps of:

(a) sizing a paperboard suitable for use as a food container;

(b) applying a base coat coating to one or both surfaces of the paperboard blank, the base coat coating comprising a mixture of an inorganic pigment and an acrylic latex comprising aliphatic copolymers having the following monomers:



wherein R and R<sup>1</sup> may be the same or different aliphatic hydrocarbons having one to six carbon atoms and the ratio of (i) to (ii) is in the range of 1:100 to 100:1;

(c) applying a top coat coating layer to the base coat coating layer, the top coat coating layer comprising an inorganic pigment and an aliphatic polymer latex comprising aliphatic copolymers having the following monomers:



wherein R and R<sup>1</sup> may be the same or different aliphatic hydrocarbons having one to six carbon atoms and the ratio of (i) to (ii) is in the range of 1:100 to 100:1; and wherein said coated container at a temperature in excess of 430° F. evolves less than 0.1 milligrams of benzene per square inch of the board surface while exposed to microwave.

30. The process of claim 29 wherein R and R<sup>1</sup> are —CH<sub>3</sub> groups and the paperboard container evolves less than 0.04 milligrams of benzene per square inch of the container surface at a temperature in excess of 430° F.

31. The process of claim 29 or claim 30 wherein the base coat and top coat are copolymer latex comprising comonomers of vinylacetate and butylacrylate.

32. The process of claim 29 or claim 30 wherein the base coat and top coat are copolymer latex comprising comonomers of vinylacetate and acrylate.

33. The process of claim 29 or claim 30 wherein the base coat is a copolymer latex comprising vinylacetate and acrylate comonomers and the top coat is a copolymer latex comprising comonomers of vinylacetate and butylacrylate.

34. The paperboard of claim 29 or claim 30 wherein the base coat is a copolymer latex comprising comonomers of vinylacetate and butylacrylate and the top coat is a copolymer latex comprising vinylacetate and acrylate comonomers.

35. The process of claim 29 or claim 30 in which the weight of the paperboard blank is controlled within the range of about 100 to 400 lbs. per 3000 square foot ream and the caliper is controlled to be in the range of about 0.008 to 0.055 inch.

36. The process of claim 35 wherein the caliper of the paper blank is controlled to be in the range of about 0.008 to 0.050 inch.

37. The process of claim 36 comprising introducing a controlled amount of moisture into the blank to produce a moisture content of about 4.0 to 12.0% by weight.

38. The process of claim 29 or claim 30 wherein the paperboard container is coated on one side with a metalized polyester to provide a food container with a microwave susceptor layer.

39. The process of claim 38 wherein the metal is aluminum.

40. The process of claim 38 wherein the metal is nickel.

41. The process of claim 38 wherein the metal coating is selected from the group consisting of aluminum, iron, nickel, copper, silver, carbon, stainless steel, nichrome, magnetite, zinc, tin, tungsten, titanium and mixtures of these.

42. The paperboard of claim 1 or claim 2 wherein the paperboard evolves less than 0.03 milligrams of benzene per square inch of the board surface at a temperature in excess of 430° F.

43. The paperboard of claim 1 or claim 2 wherein the paperboard evolves less than 0.02 milligrams of benzene per square inch of the board surface at a temperature in excess of 430° F.

44. The paperboard of claim 1 or claim 2 wherein the paperboard evolves less than 0.01 milligrams of benzene per square inch of the board surface at a temperature in excess of 430° F.

45. The paperboard container of claim 9 or claim 10 wherein the paperboard container evolves less than 0.03 milligrams of benzene per square inch of the paperboard container surface at a temperature in excess of 430° F.

46. The paperboard container of claim 9 or claim 10 wherein the paperboard container evolves less than 0.02 milligrams of benzene per square inch of the paperboard container surface at a temperature in excess of 430° F.

47. The paperboard container of claim 9 or claim 10 wherein the paperboard container evolves less than 0.01 milligrams of benzene per square inch of the paperboard container surface at a temperature in excess of 430° F.

\* \* \* \* \*